

## UNITED STATES PATENT OFFICE

2,153,134

## YARN TREATING PROCESSES AND COMPOSITIONS THEREFOR

Joseph B. Dickey and James G. McNally, Rochester, N. Y., assignors to Eastman Kodak Company, Rochester, N. Y., a corporation of New Jersey

No Drawing. Application November 26, 1937.  
Serial No. 176,682

22 Claims. (Cl. 28—1)

This invention relates to the conditioning of textile yarns and more particularly to the conditioning of filaments and yarns composed of organic derivatives of cellulose such as cellulose acetate, cellulose acetate propionate, cellulose acetate butyrate, etc., to render them more amenable to textile operations such as knitting and the like.

As is well known in the manufacture of yarns, particularly those composed of or containing cellulose organic derivatives, it is necessary to treat the yarn in order to reduce the tendency toward breakage of the individual filaments or fibers when they are subjected to various mechanical strains and to lubricate the yarn in order to facilitate handling in such operations as spinning, twisting, winding and reeling. It is also necessary to treat yarn to adapt it for use as warp or filling or for the manufacture of various types of knitted fabrics. In knitting, it is particularly important that the yarn be soft and pliable in order that it may conform readily to the contour of the needles and thus produce a closely knit fabric free from such defects as "stitch distortion", "pin holes", "laddering", and the like.

Heretofore it has been proposed to employ softening agents such as polyhydric alcohols and similar agents as ingredients of yarn conditioning or lubricating formulas, generally in connection with mineral, animal or vegetable oils. It has been found, however, that most of the known softening agents and the various formulas containing them have certain drawbacks, one of the most serious of which is high vapor pressure, and in some cases too drastic a solvent action on the yarn. Many of such agents possess slight or insufficient solvent power for the lubricants with which they are used, and it is accordingly necessary to employ blending agents or emulsifying agents in order to obtain operable yarn treating formulas. In addition, many of the known softening and lubricating agents are insufficiently soluble in water to permit satisfactory removal by aqueous scour baths.

This invention has as its principal object to provide an entirely new class of yarn conditioning agents which are particularly adapted for the treatment of yarn composed of or containing organic derivatives of cellulose and capable of lubricating, softening and rendering such yarns more amenable to knitting and other textile operations. A further and specific object is to provide a class of conditioning agents which augment or assist the lubricating action of various lubricants when applied to such yarns. A still

further object is to provide yarn softening and lubricating formulas which can be readily removed from the yarns by the usual scour baths. A still further object is to provide an improved method for the conditioning of yarns, particularly those composed of or containing organic derivatives of cellulose such as cellulose acetate, whereby the yarn is rendered soft and pliable and capable of employment in a variety of textile operations where complicated designs or stitches are employed. Still another object is to provide new chemical compounds having the structure and properties discussed below. Another object is to provide an improved type of yarn which is especially amenable to textile operations including knitting, weaving, spinning, and the like. Other objects will appear hereinafter.

These objects are accomplished by the following invention which in its broader aspects comprises the discovery that acetals having the general formulas:



5

10

15

15

20

25

30

35

35

40

45



where R and R' may be hydrogen, alkoxy or alkyl and tetrahydrofurfuryl groups, may be used as yarn conditioning agents and particularly as softening agents, with or without the addition of animal, mineral, or vegetable oils, in the treatment of yarns composed of or containing organic derivatives of cellulose. We have found that these compounds have a slight solvent and/or softening action on cellulose organic derivative yarns which renders such yarns soft and pliable without at the same time having too drastic a solvent action thereon.

In accordance with the invention these compounds may be applied directly to the yarn during or after spinning, or may be added to the spinning solution itself. We have found that these compounds have exceptional solvent powers which enable them to dissolve mineral oils and blown and unblown, drying and semi-drying, vegetable and animal oils and accordingly they may be, and preferably are, employed as ingredients of yarn conditioning or lubricating formulas in conjunction with agents which function wholly or partially as lubricants.

In the following examples and description we

25

30

35

40

45

50

55

have set forth several of the preferred embodiments of our invention, but they are included merely for purposes of illustration and not as a limitation thereof.

5 The compounds which we have found particularly valuable for treating yarn in accordance with the process herein described may be prepared in accordance with the general methods outlined in the literature as follows:

10 Preparation of acetals using acetylene and alcohols

—Nieuwlands, J. Amer. Chem. Soc. 45, 1552 (1923)

Furfural cyclic acetals

15 —U. S. Pat. 1,934,309

Hydrogenation of furfural acetals

—Minnie and Adkins, J. Amer. Chem. Soc. 55, 299 (1933)

—Adkins, *Ibid.*, 54, 1651 (1932)

20 In order to illustrate the preparation of compounds in accordance with our invention, the following examples are given:

Preparation of



One gram of red mercuric oxide is partially dissolved by gentle warming in 5 grams of 50% 30 boron trifluoride in methanol. Tetrahydrofurfuryl alcohol (102 grams; 1 mol) is then added, the flask placed in cold water, and the mixture treated with dry acetylene until the theoretical quantity is absorbed (13 grams). The flask and 35 contents are shaken frequently during the addition. A further 1 gram of  $HgO$  is added as the reaction becomes slow.

Preparation of tetrahydrofurfural glycol

40 Five hundred sixty four grams (4 mols) furfural glycol, 5 grams isoamylamine, and 20 grams Raney catalyst are treated with hydrogen at 150° under 1500 pounds pressure for 20 hours. The product is worked up by known methods to give 45 400 grams (70%) of reduced compounds, B. P. 14 87-95°. In an exactly similar manner there may be prepared:



and



Preparation of tetrahydrofurfural formal

A mixture of 204 grams tetrahydrofurfuryl alcohol (2 mols), 40 grams trioxymethylene (.45 mol), and 1 cc. conc. sulfuric acid are gently refluxed for six hours. After 15 minutes all the para-formaldehyde has gone into solution. The reaction is allowed to stand overnight at room temperature and then neutralized with excess sodium carbonate, filtered and distilled. B. P. 10 60-165°; refr. index 1.4583 at 24°; sp. gr. 1.075 at 24°.

70 Our invention will be more readily understood by reference to the following examples in which typical applications of the invention are set forth.

Example I.—A 20% solution of cellulose acetate in acetone in which is incorporated

1-25% by weight of the cellulose acetate of tetrahydrofurfural glycol



is extruded through fine orifices into an evaporative atmosphere. The filaments thus produced are wound or twisted and wound. Yarns produced from filaments thus prepared are pliable 10 and suitable for knitting.

Example II.—Yarn composed of cellulose acetate and designed for knitting purposes is treated by applying thereto tetrahydrofurfural glycol



by means of an applicator roll. The amount of 20 the conditioning liquid may run from 4-25% by weight of the yarn. If the yarn is intended for weaving, the same procedure may be followed except that the amount of the conditioning agent added to the yarn is about 1-5%.

Example III.—A conditioning liquid is made up by mixing the following ingredients in the indicated proportions:

Ditetrahydrofurfuryl acetal..... 70 parts 30



Olive oil..... 30 parts 35

This composition is applied to a cellulose acetate yarn intended for knitting in an amount representing 4-25% by weight of the untreated yarn. The filaments or fibers thus treated are quite soft and pliable and give excellent results in 40 textile operations, especially knitting.

Other examples of yarn conditioning compositions which may be applied to various types of yarn, particularly cellulose acetate, cellulose acetate propionate, and similar cellulose organic 45 derivative yarns in accordance with our invention and which render such yarns soft and pliable and well-adapted for various textile operations, particularly knitting, are the following:

Example IV

Ditetrahydrofurfuryl acetone..... 60 parts



Blown olive oil..... 40 parts

Example V

Ditetrahydrofurfuryl tetrahydrofuran..... 70 parts 60



Neat's-foot oil..... 30 parts

Example VI

Ditetrahydrofurfuryl -  $\beta$  - methoxyethyl..... 70 parts 70



Blown neat's-foot oil..... 30 parts 75

## Example VII

|                           | Per cent |
|---------------------------|----------|
| Tetrahydrofurfural glycol | 70       |
| Light mineral oil         | 30       |

5

## Example VIII

|                                        | Per cent |
|----------------------------------------|----------|
| Tetrahydrofurfuryl trimethylene glycol | 50       |
| Sperm oil                              | 50       |

10

## Example IX

|                             | Per cent |
|-----------------------------|----------|
| Ditetrahydrofurfuryl acetal | 70       |
| Blown sperm oil             | 30       |

15

## Example X

|                             | Parts |
|-----------------------------|-------|
| Ditetrahydrofurfuryl formal | 30    |
| Blown teaseed oil           | 70    |

20

## Example XI

|                                      | Parts |
|--------------------------------------|-------|
| Tetrahydrofurfural diethylene glycol | 40    |

25



30

## Example XII

|                              | Parts |
|------------------------------|-------|
| Ditetrahydrofurfurylfurfural | 60    |
| Blown neat's-foot oil        | 40    |

As will be apparent from the above examples and description, the conditioning agents of our invention may be applied by a wide variety of methods. For example, we may employ the agent as an ingredient of the spinning dope from which the filaments are formed, the amount of the agent so employed depending upon a number of factors, such as the particular cellulose derivative used in making the yarn, the solvent or solvent combination used in making up the spinning solution, and the degree of softness or pliability desired in the yarn, etc.

If the conditioning agent is to be applied to the yarn after spinning, this may be done by bringing the yarn in contact with a wick, roll, or felt wet therewith or the liquid may be applied by immersion, spray, or otherwise. The particular point at which the liquid is applied may vary. It may, for example, be applied to the yarn inside or outside the spinning cabinet, between the guide and godet roll, between the godet or other roll or guide and the point of winding and/or twisting. In some cases, the liquid may even be applied to the yarn after winding onto cones, spools, bobbins, or the like or by the so-called "bobbin to bobbin" method. In the case of staple fiber manufacture, the liquid may be applied to the yarn prior to, or after cutting into staple lengths.

The amount of the agent so employed will vary widely depending upon the results desired, the specific nature of the material to which the agent is applied, the use to which the yarn is eventually to be put and other factors. For example, in a given case where a cellulose organic acid ester yarn such as a yarn composed of cellulose acetate, is intended for knitting, about 4 to 25% or more by weight, based on the weight of the dry yarn, may be satisfactory, while if the yarn is intended for weaving, the amount may vary between about 1 and 5%.

Although in the above examples we have referred primarily to yarn treating compositions containing only the conditioning agent and an

oil, other ingredients such as solvents, non-solvents emulsifying agents, blending agents and the like, may be added within the scope of our invention. Likewise, various dyes or other coloring matter may be included in case it is desired to permanently or fugitively tint or dye the material undergoing treatment.

Although we have found it convenient to illustrate our invention by reference to compositions containing specific percentages of the various ingredients, these percentages may vary widely depending upon the particular purpose for which the composition is intended. For example, if it is desired to control the solvent or softening action of the conditioning agent, the amount of the agent may be adjusted as, for example, by reducing the amount of the agent and correspondingly increasing the amount of oil or other ingredient.

While we have described our invention with particular reference to the treatment of yarns composed of organic derivatives of cellulose such as cellulose acetate, the conditioning agents and formulas described herein are applicable to the conditioning of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others, as well as to the conditioning of silk, wool, cotton, viscose and other natural or artificial materials.

The term "yarn" as used herein and in the claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

As indicated above, the yarn conditioning agents of our invention are exceptionally good solvents for a wide variety of mineral, blown and unblown, drying and semi-drying animal and vegetable oils such as cottonseed, olive, castor, neat's-foot, sperm and other oils. This enables them to be used with any of such oils in making up a variety of yarn treating formulas of varying composition.

The yarn conditioning method and compositions of our invention possess many outstanding advantages. The fundamental and outstanding characteristics of the agents employed in accordance with the invention is their ability to soften yarns, especially those composed of or containing organic derivatives of cellulose such as cellulose acetate and render them soft and pliable and amenable to various textile operations, especially operations such as those involved in weaving and knitting where complicated designs or stitches are employed, without too drastic an action on the yarn material. Another outstanding characteristic of these compounds is their exceptional solvent power for a wide variety of mineral, animal and vegetable oils and their ability to act as lubricating assistants in conjunction with these oils when applied to such yarns. In addition, due to their solubility in water, they may be readily removed from yarns and fabrics by means of the usual aqueous scour baths. By employing the yarn conditioning agent and method

of our invention as herein described, one is enabled to obtain highly satisfactory results in the manufacture of yarns and woven fabrics and especially the production from these yarns of closely knit fabrics free from defects such as pin holes, stitch distortion, laddering and the like.

What we claim and desire to secure by Letters Patent of the United States is:

1. The process of conditioning yarn to render it more amenable to textile operations including knitting, weaving, spinning, and the like which comprises applying thereto a lubricating and softening composition containing as its essential lubricating and softening components an acetal selected from the group consisting of acetals having the formulas:



20 and



25 where R and R' is a substituent selected from the group consisting of hydrogen, alkoxy and alkyl and tetrahydrofurfuryl.

2. The process of conditioning yarn composed of or containing organic derivatives of cellulose to render it more amenable to textile operations including knitting, weaving, spinning and the like which comprises applying thereto a lubricating and softening composition containing as its essential lubricating and softening compound an acetal selected from the group consisting of acetals having the formulas:



40 and



45 where R and R' is a substituent selected from the group consisting of hydrogen, alkoxy and alkyl and tetrahydrofurfuryl.

3. The process of conditioning yarn composed of or containing cellulose acetate to render it more amenable to textile operations including knitting, weaving, spinning and the like, which comprises applying thereto a lubricating and softening composition containing as its essential lubricating and softening component an acetal selected from the group consisting of acetals having the formulas:



60 and



65 where R and R' is a substituent selected from the group consisting of hydrogen, alkoxy and alkyl and tetrahydrofurfuryl.

4. The process of conditioning yarn composed of or containing cellulose acetate to render it more amenable to textile operations including knitting, weaving, spinning and the like, which comprises applying thereto a lubricating and softening composition containing as its essential

lubricating and softening component an acetal selected from the group consisting of acetals having the formulas:



5

and



10

where R and R' is a substituent selected from the group consisting of hydrogen, alkoxy and alkyl and tetrahydrofurfuryl and a textile lubricant.

5. The process of conditioning yarn composed of or containing cellulose acetate to render it more amenable to textile operations including knitting, weaving, spinning and the like, which comprises applying thereto a lubricating and softening composition containing as its essential lubricating and softening component the cellulose acetate of tetrahydrofurfural glycol.

6. The process of conditioning yarn composed of or containing cellulose acetate to render it more amenable to textile operations including knitting, weaving, spinning and the like, which comprises applying thereto a lubricating and softening composition containing as its essential lubricating and softening component ditetrahydrofurfuryl acetal.

7. The process of conditioning yarn composed of or containing cellulose acetate to render it more amenable to textile operations including knitting, weaving, spinning and the like, which comprises applying thereto a lubricating and softening composition containing as its essential lubricating and softening component ditetrahydrofurfuryl tetrahydrofurfural.

8. A conditioning agent for rendering yarns more amenable to textile operations including knitting, weaving, spinning, and the like which comprises an acetal selected from the group consisting of acetals having the formulas:



45

and



50

where R and R' is a substituent selected from the group consisting of hydrogen, alkoxy and alkyl and tetrahydrofurfuryl.

9. A conditioning agent for rendering textile yarns composed of or containing organic derivatives of cellulose more amenable to textile operations including knitting, weaving, spinning, and the like which comprises an acetal selected from the group consisting of acetals having the general formulas:



65

and



70

where R and R' is a substituent selected from the group consisting of hydrogen, alkoxy and alkyl and tetrahydrofurfuryl and a textile lubricating oil.

75

10. A conditioning agent for rendering yarns composed of or containing cellulose acetate more amenable to textile operations including knitting, weaving, spinning and the like containing the cellulose acetate of tetrahydrofurfural glycol.

11. A conditioning agent for rendering textile yarns composed of or containing cellulose acetate more amenable to textile operations including knitting, weaving, spinning and the like containing ditetrahydrofurfuryl acetal.

12. A conditioning agent for rendering textile yarns composed of or containing cellulose acetate more amenable to textile operations including knitting, weaving, spinning and the like containing ditetrahydrofurfuryl tetrahydrofurfural.

13. Textile yarn amenable to textile operations including knitting, weaving, spinning and the like impregnated with a lubricant containing an acetal selected from the group consisting of acetals having the formulas:



26 and



28 where R and R' is a substituent selected from the group consisting of hydrogen, alkoxy and alkyl and tetrahydrofurfuryl.

14. Textile yarn composed of or containing organic derivatives of cellulose amenable to textile operations including knitting, weaving, spinning and the like, impregnated with a conditioning agent comprising an acetal selected from the group consisting of acetals having the formulas:



40 and



45 where R and R' is a substituent selected from the group consisting of hydrogen, alkoxy and alkyl and tetrahydrofurfuryl.

15. Textile yarn composed of or containing organic derivatives of cellulose amenable to textile operations including knitting, weaving, spinning and the like, impregnated with a conditioning

ing agent comprising an acetal selected from the group consisting of acetals having the general formulas:



and



5

10

15

20

25

30

35

40

45

50

where R and R' is a substituent selected from the group consisting of hydrogen, alkoxy and alkyl and tetrahydrofurfuryl and a textile lubricant.

16. Textile yarns composed of or containing cellulose acetate amenable to textile operations including knitting, weaving, spinning and the like, impregnated with a lubricant comprising the cellulose acetate of tetrahydrofurfural glycol.

17. Textile yarns composed of or containing cellulose acetate amenable to textile operations including knitting, weaving, spinning and the like, impregnated with a lubricant comprising ditetrahydrofurfuryl acetal.

18. Textile yarns composed of or containing cellulose acetate amenable to textile operations including knitting, weaving, spinning and the like, impregnated with a lubricant comprising ditetrahydrofurfuryl tetrahydrofurfural.

19. As new chemical compounds acetals selected from the group consisting of acetals having the formulas:



and



35

40

wherein R and R' is a substituent selected from the group consisting of hydrogen, alkoxy, alkyl and tetrahydrofurfuryl.

20. As a new chemical compound, the cellulose acetate of tetrahydrofurfural glycol.

21. As a new chemical compound, ditetrahydrofurfuryl acetal.

22. As a new chemical compound, ditetrahydrofurfuryl tetrahydrofurfural.

JAMES G. McNALLY.  
JOSEPH B. DICKEY.

### Certificate of Correction

Patent No. 2,153,134.

JOSEPH B. DICKEY ET AL.

April 4, 1939.

It is hereby certified that error appears in the printed specification of the above numbered patent requiring correction as follows: Page 5, second column, line 5, claim 15, in the formula, for



read



and that the said Letters Patent should be read with this correction therein that the same may conform to the record of the case in the Patent Office.

Signed and sealed this 27th day of June, A. D. 1939.

Henry Van Arsdale

Acting Commissioner of Patents.

[SEAL]

10. A conditioning agent for rendering yarns composed of or containing cellulose acetate more amenable to textile operations including knitting, weaving, spinning and the like containing the cellulose acetate of tetrahydrofurfural glycol.

11. A conditioning agent for rendering textile yarns composed of or containing cellulose acetate more amenable to textile operations including knitting, weaving, spinning and the like containing ditetrahydrofurfuryl acetal.

12. A conditioning agent for rendering textile yarns composed of or containing cellulose acetate more amenable to textile operations including knitting, weaving, spinning and the like containing ditetrahydrofurfuryl tetrahydrofurfural.

13. Textile yarn amenable to textile operations including knitting, weaving, spinning and the like impregnated with a lubricant containing an acetal selected from the group consisting of acetals having the formulas:



26 and



28 where R and R' is a substituent selected from the group consisting of hydrogen, alkoxy and alkyl and tetrahydrofurfuryl.

14. Textile yarn composed of or containing organic derivatives of cellulose amenable to textile operations including knitting, weaving, spinning and the like, impregnated with a conditioning agent comprising an acetal selected from the group consisting of acetals having the formulas:



40 and



45 where R and R' is a substituent selected from the group consisting of hydrogen, alkoxy and alkyl and tetrahydrofurfuryl.

15. Textile yarn composed of or containing organic derivatives of cellulose amenable to textile operations including knitting, weaving, spinning and the like, impregnated with a conditioning

ing agent comprising an acetal selected from the group consisting of acetals having the general formulas:



and



5

10

15

20

25

30

35

40

45

50

where R and R' is a substituent selected from the group consisting of hydrogen, alkoxy and alkyl and tetrahydrofurfuryl and a textile lubricant.

16. Textile yarns composed of or containing cellulose acetate amenable to textile operations including knitting, weaving, spinning and the like, impregnated with a lubricant comprising the cellulose acetate of tetrahydrofurfural glycol.

17. Textile yarns composed of or containing cellulose acetate amenable to textile operations including knitting, weaving, spinning and the like, impregnated with a lubricant comprising ditetrahydrofurfuryl acetal.

18. Textile yarns composed of or containing cellulose acetate amenable to textile operations including knitting, weaving, spinning and the like, impregnated with a lubricant comprising ditetrahydrofurfuryl tetrahydrofurfural.

19. As new chemical compounds acetals selected from the group consisting of acetals having the formulas:



and



35

40

wherein R and R' is a substituent selected from the group consisting of hydrogen, alkoxy, alkyl and tetrahydrofurfuryl.

20. As a new chemical compound, the cellulose acetate of tetrahydrofurfural glycol.

21. As a new chemical compound, ditetrahydrofurfuryl acetal.

22. As a new chemical compound, ditetrahydrofurfuryl tetrahydrofurfural.

JAMES G. McNALLY.  
JOSEPH B. DICKEY.

### Certificate of Correction

Patent No. 2,153,134.

JOSEPH B. DICKEY ET AL.

April 4, 1939.

It is hereby certified that error appears in the printed specification of the above numbered patent requiring correction as follows: Page 5, second column, line 5, claim 15, in the formula, for



read



and that the said Letters Patent should be read with this correction therein that the same may conform to the record of the case in the Patent Office.

Signed and sealed this 27th day of June, A. D. 1939.

Henry Van Arsdale

Acting Commissioner of Patents.

[SEAL]